

June 19, 1934.

R. D. McDILL

1,963,554

RESISTOR AND PROCESS OF MAKING SAME

Filed Jan. 4, 1933

Fig. 1.



Fig. 2.



Fig. 3.



Fig. 4.



Fig. 5.



Fig. 6.



## UNITED STATES PATENT OFFICE

1,963,554

## RESISTOR AND PROCESS OF MAKING SAME

Rex D. McDill, Cleveland, Ohio

Application January 4, 1933, Serial No. 650,147

13 Claims. (Cl. 201—76)

The object of my invention is to provide an improved radio resistor and a novel process of manufacturing same. I attain the objects of my invention by the means illustrated in the accompanying drawing, in which—

5 Figure 1 is a face or plan view of a strip of material made in accordance with my invention;

10 Fig. 2 is a section on line 2—2 of Fig. 1;

Fig. 3 is a section on line 3—3 of Fig. 1;

Fig. 4 is a section similar to Fig. 3 but with the

coating applied to the woven material;

Fig. 5 is a similar detail view with the terminal soldered to the material;

15 Fig. 6 is a perspective view of the completed device; and

Fig. 7 is a perspective view of a modified form of the invention.

Like numerals designate like parts in each of 20 the several views.

Referring to the accompanying drawing, I provide warp threads 1 made from linen or other textile material which is treated before weaving by passing the material through colloidal graphite 25 in aqueous solution, or carbon of the conductive resistive type, or a mixture of both; and then drying the thread. When the warp threads are dried the material is woven by passing wire threads 2 through the threads as a weft. The 30 entire weave is about thirty inches wide and the fabric for this purpose is woven about 40 mesh. The carbon or graphite threads have a negative voltage coefficient as in all resistors of the carbon type but the wire, especially nichrome wire which 35 preferably is used as the weft, has a positive voltage coefficient so that the finished resistor has as near a voltage coefficient level as it is possible to make a cheap resistor.

I provide terminals 5 which are soldered at 40 6, the terminals having the usual apertures 7, as shown in Fig. 5. To facilitate soldering the terminals, phosphor bronze wire tinned is used as a weft.

I next take the woven material and impregnate 45 it with lacquer or enamel-like bakelite 3 in which there is in suspension graphite and carbon which is high resistant material. After that is entirely dried I coat it again with dielectric varnish or enamel 4 and then cut the strip lengthwise 50 down the center as indicated by the two sets of lines designated a—a in Fig. 1. This can be formed into a circle or strip and used as a rheostat or potentiometer. This construction has a distinct advantage over the type where the slide 55 contact rubs on the carbon because that type

soon wears out and is noisy and is not uniform in its resistance, and further the carbon type has a negative voltage coefficient, and the straight wound wire type has a positive coefficient while mine seems to equalize.

It is not essential to treat the threads before weaving as the material can be cut into strips and dipped after being woven. In such case the treating material covers the entire fabric, both threads and wire. In treating the following 65 methods may be employed. The material can be dipped in the graphite solution or carbon material in suspension in liquid form or a combination of both depending upon the resistance desired in the finished product and the quantities of each used and the strength of the solution as compared to its solvent content. The material is then thoroughly dried to drive out 70 all moisture. It can then be painted with a pyroxylin enamel like Duco or the preferred way 75 is to paint it with phenolic formaldehyde (bakelite resinoid) product in a suitable solvent such as acetone, then dry off the solvent at a low temperature, and finally polymerize the resinoid by baking at a higher temperature. If the resistors are for potentiometers or rheostats of the 80 circular type a split ring is formed before the bakelite is baked on as it would crack if bent after baking. To insure complete moisture proofing of the article, an intermediate step can be 85 taken by applying a solution of paraffine and gasoline to the dried carbon treated fabric and then evaporate the solvent before applying the Duco or bakelite.

Terminals or pig tails 7 are either soldered to 90 the ends of the resistors 8 before baking, or treating with the Duco or bakelite.

Referring to Fig. 7 of the drawing, there is illustrated a variable resistor 9 in which the wires 2 protrude out through the enamel in order to 95 form electrical contact with the sliding contact member 10 which carries the terminal 11 provided with aperture 12.

In some cases I have mixed carbon and/or graphite with the enamel before applying and it 100 also makes a very good resistor.

The material can be dipped in the graphite solution or carbon material in suspension in liquid form or a combination of both depending upon the resistance desired in the finished product 105 and the quantities of each used and the strength of the solution as compared to its solvent content. The material is then thoroughly dried to drive out all moisture. It can then be painted with a pyroxylin enamel like Duco or the pre- 110

- ferred way is to paint it with phenolic formaldehyde (bakelite resinoid) product in a suitable solvent such as acetone, then dry off the solvent at a low temperature and finally polymerize the resinoid by baking at a higher temperature. 5. The process of manufacturing a resistor consisting in weaving wire woof threads through warp threads of suitable textile material, dipping the completed fabric in graphite solution, drying the material, applying a moisture proof coating of a solution of paraffine and gasoline to the dry carbon-treated fabric, evaporating the solvent, and painting the material with a suitable enamel. 6. The process of manufacturing a resistor consisting in weaving wire woof threads through warp threads of suitable textile material, dipping the completed fabric in graphite solution, drying the material, applying a moisture proof coating of a solution of paraffine and gasoline to the dry carbon-treated fabric, evaporating the solvent, and painting the material with a suitable enamel. 7. The process of manufacturing a resistor consisting in weaving wire woof threads through warp threads of suitable textile material, dipping the completed fabric in graphite solution, drying the material, applying a moisture proof coating of a solution of paraffine and gasoline to the dry carbon-treated fabric, evaporating the solvent, and painting the material with a suitable enamel. 8. The process of manufacturing a resistor consisting in weaving wire woof threads through warp threads of suitable textile material, dipping the completed fabric in graphite solution, drying the material, painting the material with phenolic formaldehyde in a suitable solvent such as acetone, drying off the solvent at a low temperature, applying a moisture proof coating of a solution of paraffine and gasoline to the dry carbon-treated fabric, evaporating the solvent, and finally polymerizing the resinoid by baking at a higher temperature. 9. The process of manufacturing a resistor consisting in weaving wire woof threads through warp threads of suitable textile material, dipping the completed fabric in graphite solution, drying the material, painting the material with phenolic formaldehyde in a suitable solvent such as acetone, drying off the solvent at a low temperature, forming a split ring, and finally polymerizing the resinoid by baking at a higher temperature. 10. The process of manufacturing a resistor consisting in weaving wire woof threads through warp threads of suitable textile material, dipping the completed fabric in graphite solution, drying the material, painting the material with phenolic formaldehyde in a suitable solvent such as acetone, drying off the solvent at a low temperature forming a split ring, and applying a moisture proof coating of a solution of paraffine and gasoline to the dry carbon-treated fabric, evaporating the solvent, and finally polymerizing the resinoid by baking at a higher temperature. 11. A resistor consisting of fabric woven from warp threads of textile material and woof threads of wire, a coating of high resistant material, and an outer coating of lacquer covering said first mentioned coating. 12. A resistor consisting of fabric woven from warp threads of textile material and woof threads of wire, a coating of high resistant material, and an outer coating of lacquer covering said first mentioned coating, terminals soldered to the woven fabric at each end thereof. 13. A resistor consisting of fabric woven from warp threads of textile material and woof threads of wire, a coating of high resistant material and an outer coating of lacquer covering said first mentioned coating, one edge of the fabric having the ends of the wires of the fabric exposed, a longitudinally slid able contact member mounted on said edge portion of the fabric, and a terminal soldered to one end of the fabric.

REX D. McDILL.

145